

## UNITED STATES PATENT OFFICE.

MICHAEL G. CORSON, OF JACKSON HEIGHTS, NEW YORK, ASSIGNOR TO ELECTRO METALLURGICAL COMPANY, A CORPORATION OF WEST VIRGINIA.

## ALLOY.

No Drawing.

Application filed June 21, 1926. Serial No. 117,597.

The invention comprises a group of quaternary copper alloys of novel composition, having in general the mechanical properties characteristic of binary and ternary aluminum bronzes, but being decidedly more resistant to corrosion than the latter.

The alloys of the invention may be regarded as alpha aluminum bronzes into which there have been incorporated chromium and nickel. It will be understood that the alpha aluminum bronzes are compositions which contain (at room temperatures) up to about 9% of aluminum, and I find it desirable to use in the compositions of the invention an aluminum content toward this upper limit, for example between 6% and 8%.

If chromium is added to molten aluminum bronzes of the alpha type, it is found that very little of the chromium becomes alloyed with the bronze and that of this quantity only about 0.4% at most goes into solid solution, the rest being in the form of separate grainlets. For the purposes of the invention it is desirable to increase the solid solubility of the chromium. I have found that this can be done with advantageous results by incorporating nickel into the alloy. Copper-aluminum-nickel-chromium alloys containing 0.5% to about 3% of chromium in solid solution have excellent corrosion resisting properties but I prefer compositions in which the content of chromium in solid solution is about 2%. Such alloys will contain at least about 6% of nickel.

The alloys of the invention can be prepared by mixing the ingredients in any order, but I have found the following method to be advantageous. An alloy is prepared containing nickel and chromium in about the proportions desired in the final alloy, and the nickel-chromium is cast into rods. An alpha aluminum bronze of the desired aluminum content is then prepared and while molten is stirred with the nickel-chromium rods. The latter gradually dissolve in the molten bath, and the stirring is discontinued when the desired quantity of chromium has been incorporated.

The alloys of the invention are workable by the methods usually applicable to bronzes. I prefer to homogenize them by quenching from a temperature about 100° C. below its melting point, for example from about 900° C. They may be quenched from somewhat lower temperatures, however, with similar results.

Quenched specimens show, for example, a tensile strength 90,000 pounds per square inch; an elongation in two inches of 40%; and a Brinell hardness of 110. After cold-rolling the strength may be increased to 130,000 pounds per square inch; and the hardness to 220 Brinell; but the elongation will be greatly diminished, for example to 3%.

When specimens of the alloys of the invention are immersed in various mildly corrosive agents for definite periods of time, the loss in weight is found to be as much as 50% less than in the case of carefully prepared binary or ternary aluminum bronzes of equal aluminum content.

Specific proportions are given herein merely by way of illustration. Any aluminum content within the alpha range may be used. The content of chromium in solid solution may be higher than those referred to herein and an excess of nickel over that required to cause the chromium to form a solid solution may be used, but such additional quantities of these metals increase the cost of the alloy and are unnecessary for most uses. Elements which do not destroy the useful properties of the alloys, such as iron, manganese, and cobalt, and small quantities of zinc or tin, are of course not precluded.

## I claim:

1. A bronze containing a substantial quantity of aluminum not greater than about 9%; more than 0.5% of chromium in solid solution, and sufficient nickel to hold the chromium in solution.

2. A bronze having an aluminum content within the approximate range 6% to 8%; having a content of chromium greater than 0.5% and less than about 8%; and contain-

ing sufficient nickel to hold the chromium in solid solution.

3. A bronze containing aluminum 6% to 8%; chromium about 2%; and nickel about 6%.

4. The method of making a non-corrosive aluminum bronze which consists of prepar-

ing a molten bath of alpha aluminum bronze and dissolving therein, without separate fusion, an alloy of nickel and chromium.

In testimony whereof, I affix my signature.

MICHAEL G. CORSON.